

H. L. WILBER,  
ROOFING MATERIAL,  
APPLICATION FILED MAR. 8, 1917.

1,278,270.

Patented Sept. 10, 1918.

*Fig. II.*



*Fig. III.*



*Fig. III.*



INVENTOR.  
Hugh L. Wilber  
BY  
Arthur C. Brown  
ATTORNEY

# UNITED STATES PATENT OFFICE.

HUGH L. WILBER, OF KANSAS CITY, MISSOURI.

## ROOFING MATERIAL.

1,278,270.

Specification of Letters Patent. Patented Sept. 10, 1918.

Application filed March 8, 1917. Serial No. 153,287.

To all whom it may concern:

Be it known that I, HUGH L. WILBER, a citizen of the United States, residing at Kansas City, in the county of Jackson and State of Missouri, have invented certain new and useful Improvements in Roofing Material; and I do declare the following to be a full, clear, and exact description of the invention, such as will enable others skilled in the art to which it appertains to make and use the same, reference being had to the accompanying drawings, and to the letters and figures of reference marked thereon, which form a part of this specification.

My invention relates to roofing material, and more particularly to shingles, roofing strips, or the like, wherein a fibrous body is employed and to which a coating of asphalt, tar or an equivalent compound is applied to render the body water and weather proof; the principal object of the invention being to provide roofing material of this character wherein the coating compound is applied only to the exposed surface and is substantially keyed to the body to prevent its cracking or peeling therefrom, and to add strength and durability to the body strip.

In accomplishing this and other objects of the invention, I have provided improved details of structure, the preferred forms of which are illustrated in the accompanying drawing, wherein:

Figure I is a perspective view of a shingle or roofing strip embodying the present invention; the coating compound being removed from a portion of the strip to illustrate the perforated body.

Fig. II is an enlarged sectional view of the same, particularly illustrating the keying of the coating compound to the body strip.

Fig. III is a plan view of the under side of a portion of the strip showing the key heads.

Referring more in detail to the drawings:

1 designates a sheet of roofing material constructed according to the present invention, comprising a body strip 2, of an absorbent fibrous material, such as rag or wool felt, or such paper products commonly known as straw board, chip board, flax board or any other fibrous material, to which is applied a mastic durable coating 3 of waterproofing compound consisting of asphal-

tum, tar, or an equivalent, which is applied when in a liquid state to the web to give the latter strength and to render it weather proof.

In preparing the body strip, or web, 2, it is provided throughout its entire surface with closely spaced perforations 4 which are preferably arranged in staggered rows so as not to impair the strength of the strip, and are preferably of such size as to comprise about one-half of the area of the strip. The apertures are preferably punched from the material to leave the perforations entirely open so that they may readily receive the coating compound.

Before applying the surface coating 3 to the web the latter is first drawn through a liquid preservative compound so that not only the web surfaces become saturated, but the compound enters the perforations and effects almost instant saturation of the web.

After being saturated by the preservative compound, the web is drawn between rollers where all the superfluous liquid is squeezed out and the web left ready to receive the outer coating 3.

The strip of fabric is then passed into a vat where the mastic coating is applied to the upper surface to waterproof the material. This coating compound, consisting chiefly of asphalt, or tar, is applied when in a liquid state and is rolled or ironed over the surface of the web to produce a coating of uniform thickness and to press the material into the apertures 4 to form the key members 5 and the key heads 6 which overlap the under surface of the web about the edges of the apertures and serve, after the coating material has become dry, to securely bind the coating compound and body web together.

Before the coating has become thoroughly dry, grit or sand 7 may be sifted over the surface and pressed thereinto to provide a more durable wearing surface for the material.

Assuming that the material is prepared in this manner it will be seen that the coating is applied only to one side of the web, that being the side which is to be exposed to the weather, while the apertures in the web permit a more thorough saturation and also provide means for substantially keying the coating to the web so that climatic conditions will not cause cracking or peeling of the coating from the body.

It is also apparent that the key heads will effectively hold the outer coating to the body and that a coating of greater thickness than is customary may be applied. It is also noted that the perforated body is substantially strengthened by the keys so that a durable and substantial product is provided.

Having thus described my invention, what I claim as new therein, and desire to secure by Letters-Patent, is:—

Roofing material comprising a perforated

sheet of absorbent material coated on one side only with a bituminous material, the said material projecting through perforations in the sheet with the projecting portions spread on the uncoated side of the sheet to form a plurality of individual keys whereby the covering material is bonded to the perforated sheet, substantially as set forth.

In testimony whereof I affix my signature.

HUGH L. WILBER.